

Nov. 11, 1941.

M. FAIRLIE ET AL

2,262,529

LUBRICATION

Filed July 15, 1938



Fig. 2.



INVENTORS  
Matthew Fairlie  
Leonard E. Beare  
BY

Davis, Davis, Dawson and Lamondes  
ATTORNEYS

## UNITED STATES PATENT OFFICE

2,262,529

## LUBRICATION

Matthew Fairlie and Leonard E. Beare, Hammond, Ind., assignors to Sinclair Refining Company, New York, N. Y., a corporation of Maine

Application July 15, 1938, Serial No. 219,459

7 Claims. (Cl. 123—196)

This invention relates to lubrication and particularly to lubrication employing petroleum-base oils containing aluminum soaps. The invention aims to prolong the useful life of such oils, inhibit formation of "carbon," sludge, tars, asphaltenes and other injurious products in such oils during service, and to substantially reduce piston lacquering, ring-sticking, etc., in internal combustion engines and the like in which the petroleum-base oils containing aluminum soaps are used. The invention also aims to reduce corrosion of metal parts, particularly bearings, with which the oil comes in contact.

As described and claimed in our co-pending application, Serial No. 219,457, filed July 15, 1938, we have discovered that if petroleum-base oils, either compounded or uncompounded, are heated substantially above normal crank case temperature and passed in contact with a solid selected from the group consisting of the alkaline earth metals and their inorganic compounds, the tendency for the oil to deteriorate during service is reduced and difficulties due to ring-sticking, etc., are inhibited. In our co-pending application, Serial No. 219,458, filed July 15, 1938, we have described and claimed a further discovery, to wit, that mixtures containing more than one of the three alkaline earth metals or their inorganic compounds, are more effective as a contact mass for inhibiting deterioration of petroleum base oils and inhibiting corrosion of metals with which the oils come in contact than a contact mass containing only one of the alkaline earth metals in elemental or combined form. In a third co-pending application, Serial No. 219,456, filed July 15, 1938, we have described and claimed our discovery that contact masses of alkaline earth metals or inorganic compounds thereof are very effective in preventing deterioration of and corrosion by petroleum-base oils containing a soap of an alkaline earth metal even at normal crank case temperatures and below. By analogy, it would seem that aluminum or its inorganic compounds might be used as a contact mass to inhibit deterioration of and corrosion by petroleum base lubricating oils containing aluminum soaps. We have discovered, however, that aluminum and its compounds are not useful in this respect, but that the deterioration of and corrosion by petroleum oils containing aluminum soaps are inhibited substantially even at relatively low temperatures if the oil is brought repeatedly into contact with a solid selected from the group consisting of the alkaline earth metals and inorganic compounds thereof. The bene-

ficial effects of such treatment are, however, augmented at elevated temperatures. Our invention, therefore, contemplates a method of treating a petroleum-base lubricant which comprises passing said lubricant containing an aluminum soap in repeated contact with a solid selected from the group consisting of the alkaline earth metals and inorganic compounds thereof. Preferably, the solid is in porous or finely divided form so that the oil may be forced through it. Thus, the solid or "contact mass" may be in the form of a filter disposed in the lubricating system of an internal combustion engine, the oil being pumped out of the service zone of the system, for example, the crank case of the engine through the filter and back into the service zone.

All of the alkaline earth metals, i. e., calcium, barium, and strontium, may be employed in the practice of our invention either in metallic form or as inorganic compounds, for example the hydroxides, oxides, carbonates and carbides. The hydroxides are preferable from an economic standpoint, because they are both efficacious and relatively inexpensive.

In the preferred practice of our invention, the oil containing the aluminum soap is withdrawn from a service zone, for example the crank case of an internal combustion engine, brought to optimum treatment temperature, which in general is in excess of about 240° F. and preferably about 300° F., and then circulated back to the service zone through a contact mass of porous hydroxide of calcium, barium or strontium. In general, the higher the rate of circulation, the better are the results obtained, but good results have been obtained with a porous contact mass weighing about 200 gm. grams (or about 20% of the weight of the oil in circulation) through which the oil was circulated at the rate of 150 ccs. per minute (or approximately 15% of the total oil in the system per minute).

The beneficial action of the contact mass apparently is directly proportional to the exposed surface of the active ingredient, for example, strontium hydroxide. Consequently, the contact mass should be as porous or as finely divided as possible, consistent with the limitations imposed by the necessity of forcing the oil through the mass by a reasonable degree of pressure and without having the particles so fine that a substantial amount of them are entrained by the oil and carried into the service zone where, conceivably, they may bring about abrasion. In general, however, we have found that it is not

desirable to employ a mass in which a substantial proportion of the particles are larger than pea size or smaller than about 14 mesh.

The contact mass may be in the form of a coherent body of particles that have been caused to adhere or cohere in any appropriate manner, or it may be in the form of loose particles of appropriate size retained in a pervious-walled receptacle, say, a canister made of metal screen or perforated metal plate, or a fabric bag.

Our invention will be more thoroughly understood in the light of the following detailed description taken in conjunction with the accompanying drawing, in which:

Fig. 1 is a vertical section through a filter mechanism adapted for holding the contact mass, the connection of the filter to the lubricating system of an internal combustion engine being shown schematically, and

Fig. 2 is a graph of results obtained in testing cadmium-silver bearings in a laboratory bearing corrosion test machine lubricated with a petroleum-base oil containing an aluminum soap, in one case employing a contact mass of calcium hydroxide through which the oil was circulated, and in another case which was similar in all respects except that no contact mass was employed.

Passing now to a consideration of the drawing, the filter of Fig. 1 comprises a cylindrical metal shell 10 having a cover plate 11 bolted to a flange 12 around the top of the shell with a gasket 13 interposed between the flange and the top to insure a tight joint. Disposed concentrically within the shell is a canister 14 made from perforated Monel metal screen or other pervious corrosion-resistant material. The canister is annular in form with an enclosing top portion 15 so that it surrounds a space 16 immediately above an outlet pipe 17. An inlet pipe 18 is provided in the outside of the shell and the space in the shell around the canister is filled with cotton wool 19. The inside of the canister is filled with a pervious mass of an inorganic solid 20, containing calcium, strontium or barium in elemental or combined form. Thus, the canister may be packed with twisted calcium foil, but for economic reasons, it is desirable to fill the canister with fine lumps (say 8 to 14 mesh) of the hydroxide or carbide of an alkaline earth metal or a mixture of the two. An oil containing aluminum soap is withdrawn from the crank case of the engine and by means of a pump forced through the cotton wool and the contact mass of alkaline earth metal or inorganic compound thereof to the outlet. From the outlet the treated oil is returned to the crank case so that a repeated circulation is set up.

The tendency of the contact mass to escape from the filter is relatively slight. Lumps of calcium hydroxide and the like are relatively friable in the air, but when once wetted with oil there is little tendency for them to break apart. However, the cotton wool is provided as a safeguard against the circulation of calcium hydroxide and other solids through the engine. The cotton also serves to distribute the oil through the filter and thus prevent channeling.

As a further precaution against the escape of the contact mass into the engine, it is advisable to soak the mass with oil prior to installing the filtering on the engine. This may be done conveniently by pumping oil through the mass, so that fine particles which tend to escape may be removed prior to placing the mass in service in the lubricating system.

Fig. 2 illustrates the effectiveness of our inven-

tion in reducing corrosion of cadmium-silver bearings by a petroleum base oil containing an aluminum soap. The oil employed was a commercial product having a Saybolt viscosity of

5 56-58 at 210° F., and containing approximately 1.33% of an aluminum soap, in this case, curve A shows the progressive corrosion which resulted when this oil was circulated through a filter in which the contact mass had been replaced by 10 glass beads. Curve B shows the results obtained under exactly similar conditions and with the same oil except that a contact mass of calcium hydroxide was placed in the filter so that the oil was passed in repeated circulation with both bearing and contact mass. In both cases, the oil was circulated at a temperature of 300° F. for 32 hours, when the temperature was raised to 350° F., and the circulation continued for 8 hours more. In both cases the quantity of oil in circulation was 1.0 liter, and it was circulated at the rate of 150 ccs. per minute. In the second case, the weight of calcium hydroxide in the filter was 200.0 grams.

As shown in Fig. 2, corrosion of the cadmium-silver bearings by the oil containing the aluminum soap was very marked when no contact mass was employed and increased markedly when the temperature was increased. On the other hand, corrosion was practically completely inhibited by 25 the use of the contact mass. Moreover, the contact mass is effective in reducing sludging and the formation of tars and asphaltenes so that ring-sticking, piston lacquering and other mechanical difficulties caused by deposition of such materials tend to be diminished greatly.

We claim:

1. In the operation of a system for lubricating surfaces with a petroleum base lubricating oil containing an aluminum soap which involves repeated contacting of said oil from a body thereof with the surfaces to be lubricated and circulation of said oil through a treating zone, the improvement which comprises bringing the oil in said treating zone in contact with a solid selected 40 from the group consisting of the alkaline earth metals and inorganic compounds thereof at a rate sufficient to bring into contact with said solid an amount of oil equivalent to a substantial part of said body of oil per minute, and controlling the temperature of the oil in said treating zone to maintain the oil in contact with said solid at a temperature approximating 240°-350° F.

2. In the operation of a system for lubricating 55 the bearing surfaces of an internal combustion engine with a petroleum base oil containing an aluminum soap which involves repeated contacting of said oil from a body thereof with the bearing surfaces of said engine and circulation of said oil through a treating zone, the improvement which comprises passing the oil containing the aluminum soap in said treating zone through a porous mass of a solid selected from the group consisting of the alkaline earth metals and inorganic compounds thereof at a rate sufficient to bring into contact with said solid an amount of oil equivalent to a substantial part of said oil body per minute, and controlling the temperature of the oil in said treating zone to maintain the oil in contact with said solid at a temperature approximating 240°-350° F.

3. In the operation of a system for lubricating surfaces with a petroleum base lubricating oil containing an aluminum soap which involves repeated contacting of said oil from a body there-

of with the surfaces to be lubricated and circulation of said oil through a treating zone, the improvement which comprises passing the oil in said treating zone through a porous mass of a solid selected from the group consisting of the alkaline earth metals and inorganic compounds thereof at a rate sufficient to bring into contact with said solid an amount of oil equivalent to a substantial part of said oil body per minute, and controlling the temperature of the oil in said treating zone to maintain the oil in contact with said solid at a temperature approximating 300° F.

4. In the operation of a system for lubricating surfaces with a petroleum base lubricating oil containing an aluminum soap which involves the repeated contacting of said oil from a body thereof with the surfaces to be lubricated and circulation of said oil through a treating zone, the improvement which comprises bringing the oil in said treating zone in contact with a solid selected from the group consisting of the alkaline earth metals and inorganic compounds thereof at a rate sufficient to bring into contact with said solid an amount of oil equivalent to at least about 15% of said oil body per minute and maintaining the oil at an elevated temperature while in contact with said solid.

5. In the operation of a system for lubricating surfaces with a petroleum base lubricating oil containing an aluminum soap which involves repeated contacting of said oil from a body thereof with the surfaces to be lubricated and circulation of said oil through a treating zone, the improvement which comprises bringing the oil in said treating zone in contact with a porous body containing substantial proportions of calcium hydroxide at a rate sufficient to bring into contact with said porous body an amount of oil equivalent to a substantial part of said oil body per minute, and controlling the temperature of

the oil in said treating zone to maintain the oil in contact with said porous body at a temperature approximating 240°-350° F.

6. In the operation of a system for lubricating a moving part of a machine with a petroleum base lubricating oil containing aluminum soap which involves repeated contacting of said oil from a body thereof with the moving parts to be lubricated and circulation of said oil through a treating zone while in service, the improvement which comprises bringing the oil containing aluminum soap in said treating zone into contact with a porous body containing a substantial proportion of barium hydroxide at a rate sufficient to bring into contact with said porous body an amount of oil equivalent to a substantial part of said oil body per minute, and controlling the temperature of the oil in said treating zone to maintain the oil in contact with said porous body at a temperature approximating 240°-350° F.
- 10 15 20 25 30 35 40
7. In the operation of a system for lubricating a moving part of a machine with a petroleum base lubricating oil containing aluminum soap which involves repeated contacting of said oil from a body thereof with the moving parts to be lubricated and circulation of said oil through a treating zone while in service, the improvement which comprises bringing the oil containing aluminum soap in said treating zone into contact with a porous body containing a substantial proportion of strontium hydroxide at a rate sufficient to bring into contact with said porous body an amount of oil equivalent to a substantial part of said oil body per minute, and controlling the temperature of the oil in said treating zone to maintain the oil in contact with said porous body at a temperature approximating 240°-350° F.

MATTHEW FAIRLIE.  
LEONARD E. BEARE.